

Feb. 18, 1958

W. T. BOLKCOM ET AL

2,823,992

ALLOY STEELS

Filed Nov. 9, 1956

2 Sheets-Sheet 1

**Fig. 1.**



**Fig. 3.**



INVENTORS  
WILBER T. BOLKCOM &  
WILLIAM E. KNAPP  
By Norton Leonard & Bull, Ctrs.

Feb. 18, 1958

W. T. BOLKCOM ET AL

2,823,992

ALLOY STEELS

Filed Nov. 9, 1956

2 Sheets-Sheet 2

Fig. 2.



INVENTORS

WILBUR T. BOLKCOM &  
WILLIAM E. KNAPP

*By Noelle Leonard & Bissell, Atty.*

# United States Patent Office

2,823,992

Patented Feb. 18, 1958

1

2,823,992

## ALLOY STEELS

Wilbur T. Bolckom, Allison Park, and William E. Knapp, Pittsburgh, Pa., assignors to American Metallurgical Products Company, Pittsburgh, Pa., a partnership of Pennsylvania

Application November 9, 1956, Serial No. 621,475

17 Claims. (Cl. 75—123)

This invention relates to alloy steels and a method of manufacturing them and particularly to alloy steel castings having improved impact properties, particularly at low temperatures, improved resistance to corrosion and unusual freedom from hot tears. This application is a continuation-in-part of our application Serial No. 599,284, filed June 22, 1956, which was in turn a continuation-in-part of our application Serial No. 280,226, filed April 3, 1952, and entitled "Alloy Steel."

There has long been a great need for a steel alloy having high impact properties at low temperatures and at the same time having the properties of toughness, corrosion resistance and weldability. For example, in the production of cast parts, such as railway car truck frames, bolsters, friction shoes, armor plate and other castings which are subject to frequent and severe impacts, impact properties and particularly low temperature impact properties, are of extreme importance. Ordinary steels used in the production of cast armor do not have the necessary toughness and resistance to impact without the addition of expensive and hard-to-get alloying constituents. Even with the addition of these expensive constituents, the low temperature impact properties are available and are difficult to maintain at the desired level. One of the primary disadvantages of impact resistant steels which have been heretofore used for the above-described purposes, has been their tendency to develop hot tears in the mold as is well known in the art, and this tendency has been a constant problem to the steel casting industry. The presence of crystalline inclusions has been found to accentuate hot tearing, although other factors are known to be pertinent.

We have discovered a steel alloy treated in the molten state with rare earth metals which is suitable for the manufacture of castings as well as wrought articles having surprising impact resistance at and below room temperatures, improved toughness, corrosion resistance and weldability and is characterized by fine grain microstructure with mostly round and very few or no crystalline inclusions. We have found that the alloy steel of our invention has the additional characteristic of greater than normal fluidity and that the castings formed therefrom have unusual resistance to hot tearing. We have also found a method of manufacturing such a steel alloy which will produce these characteristics.

The alloy steel of this invention may comprise broadly the following composition:

### Component:

### Percent by weight

|                   |              |
|-------------------|--------------|
| Carbon            | 0.1 to 1.8.  |
| Manganese         | 0.2 to 6.    |
| Phosphorus        | nil to 0.04. |
| Sulphur           | nil to 0.04. |
| Silicon           | 0.1 to 0.75. |
| Molybdenum        | Singly       |
| Chromium          | or in        |
| Tungsten          | combination  |
| Nickel            | nil to 5.    |
| Rare earth metals | nil to 4.    |

2

| Component—Continued | Percent by weight                                                                                                                                  |
|---------------------|----------------------------------------------------------------------------------------------------------------------------------------------------|
| Rare earth metals   | Residue from the treatment with about 0.0015% to 0.5% in the molten state after reducing the total oxide level of the molten metal to below .007%. |
| Iron                | Balance with residual impurities in ordinary amounts.                                                                                              |

It may be desirable to limit the composition of the alloy to narrower ranges for certain particular applications in which case the following concentrations of alloying elements will produce an alloy having the desirable characteristics of impact resistance at and below room temperatures as well as resistance to hot tears.

|                   |                                                                                                                                                    |
|-------------------|----------------------------------------------------------------------------------------------------------------------------------------------------|
| Carbon            | 0.15 to 0.35.                                                                                                                                      |
| Manganese         | 1.1 to 2.                                                                                                                                          |
| Phosphorus        | nil to 0.04.                                                                                                                                       |
| Sulphur           | nil to 0.04.                                                                                                                                       |
| Silicon           | 0.1 to .75.                                                                                                                                        |
| Molybdenum        | Singly                                                                                                                                             |
| Chromium          | or in                                                                                                                                              |
| Tungsten          | combination                                                                                                                                        |
| Nickel            | 0.2 to 1.                                                                                                                                          |
| Rare earth metals | Residue from the treatment with about 0.0025% to 0.5% in the molten state after reducing the total oxide level of the molten metal to below .007%. |
| Iron              | Balance with residual impurities in ordinary amounts.                                                                                              |

The term "rare earth metal" as used herein is intended to mean the elements bearing numbers 57 through 71 of the periodic table either singly or in combination and particularly: cerium, lanthanum, neodymium, praseodymium, samarium, illinium, europium, gadolinium, dysprosium, ytterbium, their alloys and compounds. These rare earth metals may be in the form commonly known as "misch metal." A mixture of rare earth metals which has proved particularly effective contains about 31.5 percent lanthanum, about 44.5 percent cerium, about 11 percent praseodymium, about 7 percent neodymium, and about 6 percent of the other rare earth metals above mentioned.

The presence of rare earth metals is critical and must be maintained substantially within the range set out above. The alloy must have had at least 0.0015% of rare earth metals added to the molten metal in order to produce the desirable characteristics of high impact resistance at and below room temperatures, resistance to hot tearing and fluidity. While a minimum of 0.0015% of rare earth addition must be maintained, we prefer to use a somewhat higher minimum under most conditions, and preferably we add not less than about 0.0025% of rare earth metals to the alloy. Greater additions of rare earth metals than 0.5% have proven deleterious to the alloy.

We have found that, in manufacturing the alloy steel of this invention, the molten steel is preferably killed in the furnace as, for example, by adding a deoxidizer such as silicomanganese, and the steel is then tapped. We prefer to maintain the final silicon content of the steel below 0.75. However, this is not critical and higher silicon contents may be desirable in some applications and our invention contemplates such higher silicon content. When the ladle is partly full, the steel is preferably further deoxidized by adding, for example,

1½ pounds of calcium silicon per ton of charge, and then the rare earth metals are preferably added within a range from about one ounce to about 5 pounds per ton of charge (additions up to 10 pounds per ton may, however, be made before deleteriously affecting the alloy), whereupon aluminum is preferably added in an amount of the order of 1 to 5 pounds per ton of charge, and then preferably a final addition of calcium silicon is made in an amount of the order of 1½ pounds per ton of charge before the ladle is completely filled.

It has been further discovered that within the range above specified the rare earth metals are effective only if the addition is made to molten steel in a basic condition and either after the total oxide level has been reduced to below about 0.007% or deoxidizers are added which will reduce the total oxide level to below about 0.007% before the rare earth metals have been dissolved in the bath. Attempts to add the rare earth metals within the stated proportions to acid steel have consistently failed, probably due to loss of the rare earth metals in the slag.

If extra hardenability characteristics are desired, boron may be added to the metal in the molten state without detrimentally affecting the rare earth effects. Preferably such boron additions should be in the area of 0.0005% to 0.005%.

It will be noted that the novel process may be carried out by adding the rare earth metals to the ladle, as basic steel is poured from the furnace; or if an acid lined furnace is used the molten steel and slag may be poured into a first ladle wherein the slag may be converted to basic condition, and the steel and slag may then be poured into a second ladle wherein the additions are made as above described.

The unusual properties of the alloy of this invention are best demonstrated by referring to tests which were made on alloys having compositions within the above ranges. The results of these tests are set forth in the tables which appear hereafter and in the accompanying drawings in which:

Figure 1 is a graph comparing the impact characteristics of the novel steel with those of substantially identical steel produced in the same manner but lacking the rare earth elements;

Figure 2 is a graph comparing the hot tear susceptibility of the novel steel with that of substantially identical steel produced in the same manner but lacking the rare earth metals; and

Figure 3 is a graph comparing the fluidity of the novel steel with that of substantially identical steel produced in the same manner but lacking the rare earth metals.

Specific examples are described as follows:

#### EXAMPLE NO. 1

Two heats were poured with the following analyses:

| Heat No. | C   | Mn   | P    | S    | Si  | Ni  | Cr  | Mo  |
|----------|-----|------|------|------|-----|-----|-----|-----|
| 1        | .27 | 1.19 | .016 | .027 | .41 | .60 | .24 | .53 |
| 2        | .27 | 1.24 | .018 | .024 | .43 | .57 | .26 | .54 |

In heat No. 1 the molten steel was killed in a basic lined induction furnace in the usual manner by adding 2½ pounds of aluminum and 3 pounds of calcium-manganese-silicon per ton of charge.

In heat No. 2 the molten steel was killed in the basic lined induction furnace in the following manner: After the usual ferrosilicon and ferromanganese additions, the steel was killed with 1½ pounds of aluminum, 2 pounds of the above-described rare earth metal mixture, and finally with 3 pounds of calcium-manganese-silicon per ton of charge.

The steel from both heats was poured into test block molds to form test plates which were identified by their

heat number plus alphabetical symbols for the respective plates and were heat treated as follows:

Plates 1-A, B, C and plates 2-A, B, C:

1700° F.—2 hr.—air cooled

1250° F.—2 hr.—air cooled

1575° F.—40 min.—water quenched

Plates 1-A and 2-A:

1010° F.—1 hr.—water quenched

Plates 1-B and 2-B:

1055° F.—1 hr.—water quenched

Plates 1-C and 2-C:

1110° F.—1 hr.—water quenched

Results of the Charpy specimens taken from the plates and tested at —40° F. were as follows:

Table I

[Heat No. 1 (1" x 6" x 10" plates).]

| Specimen No. | A (332) | B (322) | C (300) |
|--------------|---------|---------|---------|
| 1            | 20      | 24      | 32      |
| 2            | 21      | 22      | 36      |
| 3            | 24      | 23      | 35      |
| 4            | 21      | 25      | 33      |
| 5            | 23      | 25      | 34      |
| 6            | 21      | 23      | 34      |
| Avg.         | 21.7    | 23.7    | 34.0    |

[Heat No. 2 (1" x 6" x 10" plates).]

| Specimen No. | A (332) | B (322) | C (290) |
|--------------|---------|---------|---------|
| 1            | 35      | 42      | 55      |
| 2            | 35      | 42      | 54      |
| 3            | 33      | 48      | 55      |
| 4            | 35      | 47      | 54      |
| 5            | 33      | 46      | 55      |
| 6            | 35      | 44      | 56      |
| Avg.         | 34.3    | 44.2    | 54.8    |

The numbers in parentheses are hardnesses taken in Rockwell "C" and converted to Brinell.

Inclusions of the specimens of heat No. 1 were crystalline while those of heat No. 2 were round. The micro-structure of the specimens from both heats was a uniform tempered martensite.

The results of these impact tests can be compared by reference to Figure 1 of the drawings which graphically compares the impact resistance of the specimens from the two heats. It will be readily apparent by reference to the figure that the impact resistance values of the castings poured from heat No. 2 were consistently and greatly higher than the corresponding impact values of the castings poured from heat No. 1 to which the rare earth metals were not added.

It will be noted that the susceptibility to hot tearing of the steel poured from heat No. 2 was considerably less than that of the steel poured from heat No. 1 to which the rare earth metals were not added; however, this characteristic of the novel steel is more fully discussed under Example No. 3.

#### EXAMPLE NO. 2

Two heats were poured with the following analyses:

| Heat No. | C   | Mn   | P    | S    | Si  |
|----------|-----|------|------|------|-----|
| 3        | .34 | 1.57 | .016 | .036 | .41 |
| 4        | .32 | 1.68 | .014 | .031 | .51 |

Heat No. 3 was killed in a basic induction furnace in the usual manner by adding 2½ pounds of aluminum per ton of charge, and then 3 pounds of "Graphidox" per ton of charge were added. "Graphidox" is a commercial mixture of silicon, titanium and calcium, as for example, in the following proportions: 51.40 Si; 9.71 Ti; and 5.95 Ca.

Heat No. 4 was also killed in a basic induction furnace by adding 1½ pounds of aluminum per ton of charge,

then 3 pounds of "Graphidox" per ton of charge were added, and finally 2 pounds of the above-described rare earth metal mixture per ton of charge were added.

We have discovered that the presence of soluble nitrogen is critical in our alloy. We have found that the soluble nitrogen content should not exceed about 0.006%. This limit can be obtained by titanium additions preceding the rare earth addition. We have also found that the hydrogen content should not exceed about four parts per million. We have successfully reduced the hydrogen to this level by having a high rate of carbon boil—at least 30 points per hour. Any other means of removing hydrogen would of course be satisfactory.

Runners were removed from standard test blocks poured from these heats and the runners were normalized at 1650° F. for 20 minutes. All runners were tempered at 950° F. for two hours and air cooled. Pull bars were aged at 550° F. for three hours after machining.

The individual results obtained on the pull bar and Charpy specimens identified by heat number plus alphabetical symbols are tabulated in Table II below.

Table II

| Heat No. | Yield, p. s. i. | Tensile, p. s. i. | Elong., percent | Red. of Area, percent | Charpy Ft. Lbs. |         | Rt. | -40° F. |
|----------|-----------------|-------------------|-----------------|-----------------------|-----------------|---------|-----|---------|
|          |                 |                   |                 |                       | Rt.             | -40° F. |     |         |
| 3A       | 70,400          | 100,700           | 26.5            | 51.9                  | 48-48           |         |     |         |
| 3B       | 69,400          | 99,400            | 25.5            | 49.2                  | 49-50           |         |     |         |
| 3C       | 69,500          | 99,900            | 27.0            | 53.8                  | 48-48           |         |     |         |
| 3D       | 70,800          | 100,700           | 27.0            | 54.1                  | 45-46           |         |     |         |
| 4A       | 75,300          | 102,200           | 26.5            | 62.8                  | 46-51           | 18-20   |     |         |
| 4B       | 72,000          | 102,400           | 28.0            | 62.6                  | 51-46           | 23-25   |     |         |
| 4C       | 70,300          | 102,600           | 27.5            | 60.1                  | 52-45           | 22-22   |     |         |
| 4D       | 71,800          | 102,500           | 28.5            | 64.2                  | 50-54           | 20-16   |     |         |
| 4E       | 69,600          | 102,700           | 27.5            | 64.0                  | 51-48           | 23-22   |     |         |
| 4F       | 72,900          | 102,200           | 28.5            | 60.8                  | 55-58           | 24-23   |     |         |
| 4G       | 72,000          | 103,400           | 28.0            | 64.0                  | 54-46           | 25-22   |     |         |

The inclusions of heat No. 3 were crystalline, and the structure was uniform ferrite and pearlite. Heat No. 4 with the rare earth metal addition had mostly round duplex inclusions. There were a few of the pink crystalline inclusions present normally found in titanium treated steels, because the "Graphidox" addition contains some titanium. It was interesting to note that the rare earth metals were able to transform the normal crystalline inclusions to the round type but had no effect on the pink crystalline inclusions associated with titanium treated steels.

Summary of the average physical properties were as follows:

Table III

| Heat No. | Yield, p. s. i. | Tensile, p. s. i. | Elong., percent | Red. of Area, percent | Charpy Ft. Lbs. |         | Rt. | -40° F. |
|----------|-----------------|-------------------|-----------------|-----------------------|-----------------|---------|-----|---------|
|          |                 |                   |                 |                       | Rt.             | -40° F. |     |         |
| 3        | 70,000          | 100,200           | 26.5            | 52.2                  | 47.8            | 21.8    |     |         |
| 4        | 71,900          | 102,600           | 27.8            | 62.6                  | 50.7            |         |     |         |

Again it was noted that the hot tear susceptibility of the steel produced by heat 4 was considerably less than that produced by heat 3 to which the rare earth metals were not added. However, the following Example No. 3 discloses a series of heats and tests to determine accurately the effect of the rare earth metals upon the hot tear susceptibility of this type of steel.

## EXAMPLE NO. 3

The following heats were poured with the specified analyses. Each heat was killed in a basic induction furnace by adding 1½ pounds of aluminum per ton of charge; then 1 pound of the above-described rare earth metal mixture per ton of charge were added; and finally 3 pounds of Ca—Si—Mn per ton of charge were added.

| Heat No. | C   | Mn   | P    | S    | Si  |
|----------|-----|------|------|------|-----|
| F5       | .31 | 1.67 | .015 | .031 | .38 |
| F6       | .29 | 1.54 | .017 | .032 | .38 |
| F7       | .30 | 1.61 | .016 | .030 | .41 |
| F8       | .31 | 1.59 | .015 | .030 | .42 |
| F9       | .32 | 1.61 | .015 | .033 | .46 |
| F10      | .32 | 1.62 | .016 | .032 | .36 |
| F11      | .30 | 1.64 | .017 | .031 | .47 |
| F12      | .31 | 1.54 | .016 | .027 | .45 |
| F13      | .31 | 1.57 | .014 | .031 | .50 |

The following heats were also poured with the specified analyses, and the procedure was identical with that of the above-mentioned heats cited in this example, except that 2 pounds of the rare earth metal mixture per ton of charge were added.

| Heat No. | C   | Mn   | P    | S    | Si  |
|----------|-----|------|------|------|-----|
| F14      | .30 | 1.62 | .015 | .030 | .47 |
| F15      | .30 | 1.63 | .015 | .032 | .44 |
| F16      | .31 | 1.33 | .015 | .028 | .48 |
| F17      | .32 | 1.34 | .016 | .022 | .49 |
| F18      | .32 | 1.67 | .015 | .028 | .42 |
| F19      | .31 | 1.62 | .015 | .036 | .49 |
| F20      | .33 | 1.67 | .016 | .034 | .48 |
| F21      | .31 | 1.59 | .014 | .033 | .43 |
| F22      | .34 | 1.72 | .017 | .033 | .36 |
| F23      | .30 | 1.72 | .018 | .032 | .46 |
| F24      | .25 | 1.72 | .017 | .031 | .45 |

The hot tearing susceptibilities of castings poured from these heats was tested by pouring a so-called ¼ inch wall thickness hot spot cylinder casting from each heat. The same melting procedure was used in all heats, and all critical cores were made in exactly the same way and from the same mixture.

The results are shown in the following table and are compared in Figure 2 of the drawings with standard heats of the same steel without the rare earth metals.

Table IV

| Heat No. | Temp. of Steel Entering Mold (° F.) | Percent Contraction of Internal Diameter | Hot Tear Rating No. |
|----------|-------------------------------------|------------------------------------------|---------------------|
| 5        | 2,985                               | 0.88                                     | 1½                  |
| 6        | 2,885                               | 0.85                                     | 5                   |
| 7        | 2,910                               | 0.78                                     | 2                   |
| 8        | 2,720                               | 0.80                                     | 2                   |
| 9        | 2,925                               | 0.78                                     | 3                   |
| 10       | 2,985                               | 0.67                                     | 4                   |
| 11       | 2,840                               | —                                        | 4                   |
| 12       | 3,010                               | —                                        | 0                   |
| 13       | 2,810                               | 0.56                                     | 1½                  |
| 14       | 2,930                               | 0.86                                     | 1                   |
| 15       | 2,855                               | 0.76                                     | 2                   |
| 16       | 2,795                               | 0.70                                     | 1                   |
| 17       | 2,775                               | 0.70                                     | ½                   |
| 18       | 2,910                               | 0.66                                     | 0                   |
| 19       | 2,945                               | 0.67                                     | 2½                  |
| 20       | 2,745                               | 0.63                                     | 2½                  |
| 21       | 2,985                               | 0.60                                     | 2                   |
| 22       | 2,855                               | 0.53                                     | ½                   |
| 23       | 2,900                               | 0.25                                     | 5½                  |
| 24       | 2,765                               | 0.65                                     | 1                   |

The tests upon which the hot tear ratings were established are conducted as follows:

Steel from each heat is poured into a mold to form a cylinder having an external protuberance extending from end to end thereof. After the cylinder casting has cooled at room temperature, the casting is removed from the mold and any hot tearing in the protuberance is visually compared with standard cylinder casting samples which have been formed in the same manner. The standard samples have been numerically designated in direct proportion to the severity of hot tearing therein. Thus a rating of 0 indicates no hot tearing, and a rating of 1 indicates slight tearing, whereas a rating of 5 indicates severe tearing.

## 7 EXAMPLE NO. 4

The following 66,000 pound heat of steel was produced in a basic open hearth furnace with the following analysis:

| Heat No. | C   | Mn   | P    | S    | Si  | Ni   | Cr  | Mo  |
|----------|-----|------|------|------|-----|------|-----|-----|
| 25.      | .27 | 1.20 | .016 | .019 | .36 | 1.05 | .87 | .67 |

This heat was killed in the furnace by adding Si—Mn and was then tapped. When the ladle was approximately one-fourth full, 1½ pounds of Ca—Si per ton of charge were added, followed by ferrosilicon and ferromanganese for adjustment. When the ladle was approximately one-third full, 2 pounds of the above described rare earth metal mixture per ton of charge were plunged below the level of the bath, and then after the ladle was approximately half full, 2 pounds of aluminum per ton of charge were added. Finally, when the ladle was approximately five-eighths full, 1½ pounds of Ca—Si per ton of charge were added.

The molten steel was poured into molds to form test bar blocks having runners which were softened at 1250° F. for 1½ hours, plugs were then machined out of the runners and were secured to 4" and 2" Charpy blocks, whereupon the plugs were given the following heat treatments:

1700° F.—10 hrs.—air cooled

1575° F.—2 hrs.—water quenched

Tempered—2 hrs.—water quenched

The tempering temperatures for the various blocks were as follows:

| Block No. | Temperature, ° F. | Section Size, inches |
|-----------|-------------------|----------------------|
| 25-A      | 1,165             | 4                    |
| 25-B      | 1,100             | 4                    |
| 25-C      | 1,230             | 4                    |
| 25-D      | 1,165             | 2                    |
| 25-E      | 1,165             | 4                    |
| 25-F      | 1,230             | 4                    |
| 25-G      | 1,165             | 2                    |

After the final heat treatment, the plugs were removed from the blocks and hardness readings were taken by the standard method using Rockwell "C" and Brinell readings. Results were as follows:

Table V

| Block No. | Rockwell "C" Readings Center to Surface               | Direct Brinell | Rockwell "C" converted to Brinell | Average Brinell |
|-----------|-------------------------------------------------------|----------------|-----------------------------------|-----------------|
| 25-A      | 28.5—27.5—28.5—27—27—28.5—28—28—27.5—27—28—28.5       | 273            | 277                               | 275             |
| 25-B      | 31.0—31—30.5—31.5—30.0—31.5—31—31—30.5—30.5—30.5—30.5 | 293            | 299                               | 296             |
| 25-C      | 23—22—23.5—23.5—23—23—23.5—22.5—22.5—23—24—23.5—23.5  | 248            | 249                               | 249             |
| 25-D      | 28.5—28.5—27.5—28—27.5—27.5—27.5                      | 273            | 276                               | 275             |
| 25-E      | 28—28—28.5—28.5—29—29—28—29—28—29—28—28               | 277            | 280                               | 278             |
| 25-F      | 24—23.5—24—23—23.5—24.5—23—24—24—24—23.5—24—23—24     | 248            | 250                               | 249             |
| 25-G      | 29—28—28.5—28.5—27.5—28.5—28.5                        | 277            | 280                               | 278             |

number of inches the molten steel flowed through the spiral passage.

Table VIII

| Heat No. | C   | Mn   | P    | S    | Si  | Additions | Mold Entering Temp., ° F. | Spiral Fluidity (in.) |
|----------|-----|------|------|------|-----|-----------|---------------------------|-----------------------|
| 26       | .30 | 1.66 | .018 | .030 | .47 |           | 2,790                     | 17½                   |
| 27       | .30 | 1.63 | .018 | .032 | .46 | 2# Al+    | 2,790                     | 20½                   |
| 28       | .31 | 1.67 | .018 | .032 | .46 | 3# Ca-Mn- | 2,830                     | 23                    |
| 29       | .30 | 1.66 | .014 | .032 | .44 | Si.       | 2,870                     | 27                    |
| 30       | .32 | 1.62 | .015 | .031 | .40 |           | 2,890                     | 28½                   |
| 31       | .31 | 1.63 | .015 | .033 | .42 |           | 2,895                     | 29                    |
| 32       | .30 | 1.62 | .018 | .032 | .40 |           | 2,910                     | 31                    |

Charpy specimens were then removed from the center section of each plug. Results were as follows:

Table VI

| Block No. | Average Brinell | Charpy Ft. Lb., -40° F. |
|-----------|-----------------|-------------------------|
| 25-A      | 275             | 61-62-60-63             |
| 25-B      | 296             | 54-55-54-53             |
| 25-C      | 249             | 69-70-67-69             |
| 25-D      | 275             | 61-61-67-65             |
| 25-E      | 278             | 58-57-60-60             |
| 25-F      | 249             | 68-66-66-X              |
| 25-G      | 278             | 56-54-60-68             |

The average results of these tests, and a comparison of the results with standard requirements for steels of substantially identical analyses to which rare earth metals have not been added, are disclosed by the following tables from which it will be readily apparent that the impact resistance values of the steel produced by this heat were astonishingly great in view of values normally obtained.

Table VII

| Size of Section | Brinell | Charpy Ft. Lb. Required | -40° F. Obtained | Above Spec. | Percent Improved |
|-----------------|---------|-------------------------|------------------|-------------|------------------|
| 25              |         |                         |                  |             |                  |
| 4"              | 249     | 33.0                    | 68.8             | 35.8        | 108              |
| 4"              | 275     | 27.0                    | 61.5             | 34.5        | 128              |
| 4"              | 296     | 21.0                    | 54.0             | 33.0        | 157              |
| 2"              | 275     | 27.0                    | 63.5             | 36.5        | 135              |
| 4"              | 249     | 33.0                    | 66.7             | 33.7        | 102              |
| 4"              | 278     | 26.0                    | 58.7             | 32.7        | 126              |
| 4"              | 313     | 15.5                    | 47.0             | 31.5        | 203              |
| 2"              | 278     | 26.0                    | 57.5             | 31.5        | 121              |

## EXAMPLE NO. 5

The heats discussed under this example were made to determine the effect of the rare earth metal addition upon the fluidity of the molten steel, inasmuch as prior art efforts to obtain fine grained steel with very few or no elongated inclusions have resulted in greatly reduced fluidity, an undesirable characteristic for the production of satisfactory castings.

The following heats were prepared in a basic induction furnace, wherein the molten steel was killed by first adding 2½ pounds of aluminum per ton of charge and then 3 pounds of Ca—Si—Mn per ton of charge. The steel from each heat was poured into a mold containing a spiral passage connected to the gate, and the following table shows the fluidity of the steel and its entering temperature. The fluidity was tested by measuring the

The following heats were made in a basic induction furnace wherein the steel was first killed by adding  $1\frac{1}{2}$  pounds of aluminum per ton of charge; then 2 pounds of the above-described rare earth metal mixture per ton of charge were added; and then 3 pounds of Ca—Si—Mn per ton of charge were added. The fluidity of the steel was tested as above described, and the results are shown on the following table:

Table IX

| Heat No. | C   | Mn   | P    | S    | Si  | Additions                                                     | Mold Entering Temp., °F. | Spiral Fluidity (in.) |
|----------|-----|------|------|------|-----|---------------------------------------------------------------|--------------------------|-----------------------|
| 33       | .29 | 1.59 | .016 | .033 | .47 |                                                               |                          |                       |
| 34       | .28 | 1.60 | .016 | .033 | .48 |                                                               | 2,785                    | 21 $\frac{1}{2}$      |
| 35       | .31 | 1.62 | .016 | .031 | .46 |                                                               | 2,800                    | 24                    |
| 36       | .26 | 1.59 | .016 | .033 | .45 | 1 $\frac{1}{2}$ # Al+3# Ca—Mn—Si+2# Rare Earth metal mixture. | 2,815                    | 26                    |
| 37       | .31 | 1.62 | .016 | .032 | .47 |                                                               | 2,855                    | 28                    |
| 38       | .31 | 1.62 | .016 | .033 | .43 |                                                               | 2,890                    | 30 $\frac{1}{2}$      |
| 39       | .28 | 1.62 | .016 | .033 | .45 |                                                               | 2,900                    | 31                    |
|          |     |      |      |      |     |                                                               | 2,920                    | 30                    |

It will be understood that the molds used in testing the various heats were identical, and the average results are shown in Figure 3 of the drawings wherein it will be seen that the fluidity of steel to which the rare earth metals were added greatly exceeded that of substantially identical steels made in exactly the same manner but lacking the rare earth metals.

## EXAMPLE NO. 6

The test data outlined in Tables X—XII were obtained on a quenched and tempered high tensile plate steel containing several alloys and .15 carbon, .017 sulphur. The "treated" results were obtained from a large ingot treated with  $1\frac{1}{4}$  lbs. per ton of rare earth metals added in the form of  $\frac{3}{4}$  oz. balls after deoxidation to a level below 0.007% of total oxides. The "untreated" ingot was a sister one from the same heat processed in the identical manner except for the rare earth treatment. There was no sulphur reduction from the rare earth treatment. All tests were conducted on a 1" plate.

Table X.—V notch charpy

[In foot lbs.—Averages]

|                 | ° F.               | Untreated      | Treated        | Improvement, percent |
|-----------------|--------------------|----------------|----------------|----------------------|
| Transverse..... | { 10<br>-40<br>-70 | 24<br>20<br>17 | 38<br>32<br>27 | 58<br>60<br>59       |
|                 |                    |                |                | 50                   |

Table XI

|                   | ° F.               | Untreated      | Treated           | Improvement, percent |
|-------------------|--------------------|----------------|-------------------|----------------------|
| Longitudinal..... | { 10<br>-40<br>-70 | 70<br>72<br>58 | 111<br>105<br>101 | 59<br>45<br>74       |
|                   |                    |                |                   | 65                   |

Table XII.—Transition temperature

|                  | ° F. | Foot lbs. |
|------------------|------|-----------|
| Untreated.....   | 190  | 16        |
| LCA Treated..... | 235  | 18        |

Charpy V used for transition temperature in accordance with method given in transactions of ASM, vol. 47, 1955, pp. 135-153, "Tensile and impact properties of low carbon martensites," C. C. Busby, M. F. Hawks, and H. S. Paxton.

Careful consideration of the above tables shows that the alloy of this invention has low temperature impact properties which are far superior at  $-40^{\circ}$  F. than the

alloys heretofore used for the manufacture of cast armor and the like. The tables also show that the reduction of area is improved a minimum of 20%. It is also apparent that the improvement which results from the use of our alloys permits significant reductions in the amounts of those elements ordinarily added to steel to improve their toughness.

We believe that the unusual properties of our alloy

steel and the castings made therefrom are derived from the effect of the rare earth metals upon other elements in the alloy. Our researches have not indicated what the nature or character of that effect may be, however, we believe that there is a tying up and suppression of certain elements and an accentuation of the desirable properties of others. While this theory seems to be consistent with what we have observed we do not wish to bind ourselves to any theory. The fact is that the alloy steels of this invention have a surprising resistance to impact at and below room temperature and at the same time an increased resistance to hot tearing and an increased fluidity, a combination of characteristics heretofore regarded as impossible in the art.

While we have described and disclosed a preferred embodiment and practice of our invention it will be understood that it may be otherwise embodied and practiced within the scope of the following claims.

40 We claim:

1. An impact resisting steel alloy comprising about 0.1 to 1% carbon, about 0.2 to 6% manganese, about 0.1 to 0.75% silicon, nil to about 0.04% phosphorus, nil to about 0.04% sulphur, nil to about 5% of one or more of the group molybdenum, chromium and tungsten, nil to about 4% nickel, the residue from the treatment of the molten metal with about 0.0015 to 0.5% rare earth metals after reducing the total oxide to below 0.007% and the balance substantially iron with residual impurities in ordinary amounts.

2. An impact resisting steel alloy comprising about 0.1 to 1.8% carbon, about 0.2 to 6% manganese, 0.1 to 0.75% silicon, nil to about 0.04% phosphorus, nil to about 0.04% sulphur, the residue from the treatment of the molten metal with about 0.0015 to 0.5% rare earth metals after reducing the total oxide to below 0.007% and the balance substantially iron with residual impurities in ordinary amounts.

3. An impact resisting steel alloy comprising about 0.1 to 1% carbon, about 1 to 2% manganese, about 0.1 to 0.75% silicon, nil to about 0.04% phosphorus, nil to about 0.04% sulphur, about 0.2 to 0.5% chromium, about 0.5 to 1% molybdenum, about 0.5 to 1.5% nickel, the residue from the treatment of the molten metal with about 0.0025 to 0.5% rare earth metals after reducing the total oxide to below 0.007% and the balance substantially iron with residual impurities in ordinary amounts.

4. An impact resistant casting formed of a steel alloy comprising about 0.1 to 1.8% carbon, about 0.2 to 6% manganese, about 0.1 to 0.75% silicon, nil to about 0.04% phosphorus, nil to about 0.04% sulphur, nil to about 5% of one or more of the group molybdenum, chromium and tungsten, nil to about 4% nickel, the

residue from the treatment of the molten metal with about 0.0015 to 0.5% rare earth metals after reducing the total oxide to below 0.007% and the balance substantially iron with residual impurities in ordinary amounts, said casting being characterized by a fine grain microstructure with predominantly round inclusions and by resistance to hot tearing.

5. An impact resistant casting formed of a steel alloy comprising about 0.1 to 1% carbon, about 0.2 to 6% manganese, 0.1 to 0.75% silicon, nil to about 0.04% phosphorus, nil to about 0.04% sulphur, the residue from the treatment of the molten metal with about 0.0015 to 0.5% rare earth metals after reducing the total oxide to below 0.007% and the balance substantially iron with residual impurities in ordinary amounts, said casting being characterized by a fine grain microstructure with predominantly round inclusions and by resistance to hot tearing.

6. An impact resistant casting formed of a steel alloy comprising about 0.1 to 1% carbon, about 1 to 2% manganese, about 0.1 to 0.75% silicon, nil to about 0.04% phosphorus, nil to about 0.04% sulphur, about 0.2 to 0.5% chromium, about .5 to 1% molybdenum, about 0.5 to 1.5% nickel, the residue from the treatment of the molten metal with about 0.0025 to 0.5% rare earth metals after reducing the total oxide to below 0.007% and the balance substantially iron with residual impurities in ordinary amounts, said casting being characterized by a fine grain microstructure with predominantly round inclusions and by resistance to hot tearing.

7. An impact resisting steel alloy comprising about 0.1 to 1% carbon, about 0.2 to about 6% manganese, about 0.1 to 0.75% silicon, nil to about 0.04% phosphorus, nil to about 0.04% sulphur, nil to about 5% of one or more of the group molybdenum, chromium and tungsten, nil to about 4% nickel, the balance substantially iron with residual impurities in ordinary amounts, and having been treated in the molten state with about 0.0015 to about 0.5% by weight of rare earth metals after reducing the total oxide to below 0.007%.

8. An impact resisting steel alloy comprising about 0.15 to 0.35% carbon, about 1 to 2% manganese, about 0.1 to 0.75% silicon, nil to about 0.04% phosphorus, nil to about 0.04% sulphur, about 0.3 to 1% of one of the group molybdenum, chromium and tungsten, about 0.2 to 1% nickel, the balance substantially iron with residual impurities in ordinary amounts, and having been treated in the molten state with about 0.0025 to about 0.5% rare earth metals after reducing the total oxide to below 0.007%.

9. The method of producing impact resisting steel comprising the steps of pouring molten basic steel comprising about 0.1 to 1% carbon, about 0.2 to 6% manganese, about 0.1 to 0.75% silicon, nil to about 0.04% phosphorus, nil to about 0.04% sulphur, nil to about 5% of one or more of the group molybdenum, chromium and tungsten, nil to about 4% nickel and the balance substantially iron with residual impurities in ordinary amounts into a ladle while adding first a deoxidizer to reduce the total oxide level below 0.007% and then about 0.0015 to about 0.5% by weight of rare earth metals.

10. The method of producing impact resisting steel comprising the steps of killing a bath of molten basic steel comprising about 0.1 to 1% carbon, about 0.2 to 6% manganese, about 0.1 to 0.75% silicon, nil to about 0.04% phosphorus, nil to about 0.04% sulphur, nil to about 5% of one or more of the group molybdenum, chromium and tungsten, nil to about 4% nickel and the balance substantially iron with residual impurities in ordinary amounts in a furnace, pouring the molten metal into a ladle and while pouring making the following additions in the order specified to reduce the total oxide level below about 0.007%: about 1 to 2 pounds of calcium silicon per ton of metal, about 1/2 pound to about 5 pounds of rare earth metals per ton of metal; about 1 to 5 pounds of aluminum

per ton of metal and about 1 to 2 pounds of calcium silicon per ton of metal.

11. The method of producing impact resisting steel comprising the steps of producing a bath of molten steel, rendering said bath basic, deoxidizing said bath to a total oxide level below 0.007% and adding rare earth metals thereto.

12. The method of producing impact resisting steel comprising the steps of killing a bath of molten basic steel comprising about 0.1 to 1% carbon, about 0.2 to 6% manganese, about 0.1 to 0.75% silicon, nil to about 0.04% phosphorus, nil to about 0.4% sulphur, nil to about 5% of one or more of the group molybdenum, chromium and tungsten, nil to about 4% nickel and the balance substantially iron with residual impurities in ordinary amounts in a furnace, pouring the molten metal into a ladle and while pouring making the following additions to reduce the total oxide level below about 0.007%: about 2 to 4 pounds of calcium silicon per ton of metal about 1/2 pound to about 5 pounds of rare earth metals per ton of metal; and about 1 to 5 pounds of aluminum per ton of metal.

13. The method of producing impact resisting steel comprising the steps of killing a bath of molten basic steel comprising about 0.1 to 1% carbon, about 0.2 to 6% manganese, about 0.1 to 0.75% silicon, nil to about 0.04% phosphorus, nil to about 0.4% sulphur, nil to about 5% of one or more of the group molybdenum, chromium and tungsten, nil to about 4% nickel and the balance substantially iron with residual impurities in ordinary amounts in a furnace, pouring the molten metal into a ladle and while pouring making the following additions to reduce the total oxide level below about 0.007%: about 2 to 4 pounds per ton of metal of a material selected from the group consisting of ferromanganese and ferrosilicon, about 1/2 pound to 5 pounds of rare earth metals per ton of metal, and about 1 to 5 pounds of calcium, manganese silicon per ton of metal.

14. The method of producing impact resisting steel comprising the steps of killing a bath of molten basic steel comprising about 0.1 to 1% carbon, about 0.2 to 6% manganese, about 0.1 to 0.75% silicon, nil to about 0.04% phosphorus, nil to about 0.04% sulphur, nil to about 5% of one or more of the group molybdenum, chromium and tungsten, nil to about 4% nickel and the balance substantially iron with residual impurities in ordinary amounts in a furnace, pouring the molten metal into a ladle and while pouring making the following additions to reduce the total oxide level below about 0.007%: about 2 to 4 pounds of silicon alloy per ton of metal, about 0.03 pound to 5 pounds of rare earth metals per ton of metal; and about 1 to 5 pounds of aluminum per ton of metal.

15. The method of producing impact resisting steel comprising the steps of killing a bath of molten basic steel comprising about 0.1 to 1% carbon, about 0.2 to 6% manganese, about 0.1 to 0.75% silicon, nil to about 0.04% phosphorus, nil to about 0.04% sulphur, nil to about 5% of one or more of the group molybdenum, chromium and tungsten, nil to about 4% nickel and the balance substantially iron with residual impurities in ordinary amounts in a furnace, pouring the molten metal into a ladle and while pouring making the following additions to reduce the total oxide level below about 0.007%: about 2 to 4 pounds per ton of metal of a material selected from the group consisting of ferromanganese and ferrosilicon, about 0.03 pound to 5 pounds of rare earth metals per ton of metal, and about 1 to 5 pounds of calcium manganese silicon per ton of metal.

16. The method of producing impact resisting steel comprising the steps of killing a bath of molten basic steel comprising about 0.1 to 1% carbon, about 0.2 to 6% manganese, about 0.1 to 0.75% silicon, nil to about 0.04% phosphorus, nil to about 0.04% sulphur, nil to about 5% of one or more of the group molybdenum,

chromium and tungsten, nil to about 4% nickel and the balance substantially iron with residual impurities in ordinary amounts in a furnace, pouring the molten metal into a ladle and while pouring making the following additions to reduce the total oxide level below about 0.007%: about 1 to 5 pounds of aluminum per ton of metal, about 0.03 pound to 5 pounds of rare earth metals per ton of metal, and about 1 to 5 pounds of calcium silicon per ton of metal.

17. The method of producing impact resisting steel comprising the steps of killing a bath of molten basic steel comprising about 0.1 to 1% carbon, about 0.2 to 6% manganese, about 0.1 to 0.75% silicon, nil to about 0.04% phosphorus, nil to about 0.04% sulphur, nil to about 5% of one or more of the group molybdenum, chromium and tungsten, nil to about 4% nickel and the balance substantially iron with residual impurities in ordi- 10

5

nary amounts in a furnace, pouring the molten metal into a ladle and while pouring making the following additions in the order specified to reduce the total oxide level below about 0.007%: about 1 to 5 pounds of aluminum per ton of metal and about 0.03 pound to 5 pounds of rare earth metals per ton of metal.

References Cited in the file of this patent

UNITED STATES PATENTS

|           |                      |               |
|-----------|----------------------|---------------|
| 2,553,330 | Post et al. -----    | May 15, 1951  |
| 2,643,949 | Tisdale et al. ----- | June 30, 1953 |
| 2,683,661 | Tisdale et al. ----- | July 13, 1954 |

OTHER REFERENCES

The American Foundryman, December 1951, pages 45 and 46.

U. S. DEPARTMENT OF COMMERCE  
PATENT OFFICE  
**CERTIFICATE OF CORRECTION**

Patent No. 2,823,992

February 18, 1958

Wilbur T. Bolkcom et al.

It is hereby certified that error appears in the printed specification of the above numbered patent requiring correction and that the said Letters Patent should read as corrected below.

Column 1, line 38, for "available" read --variable--; line 54, for "allow" read --alloy--.

Signed and sealed this 15th day of April 1958.

(SEAL)  
Attest:

KARL H. AXLINE  
Attesting Officer

ROBERT C. WATSON  
Commissioner of Patents